

Patented Nov. 1, 1927.

1,647,491

# UNITED STATES PATENT OFFICE.

JOHN THOMAS WHITELEY, OF BROOKLYN, NEW YORK, ASSIGNOR OF ONE-HALF TO  
EDWARD JOHN SPINKA, OF NEW YORK, N. Y.

## RUSTLESS ALLOY STEEL.

No Drawing.

Application filed July 19, 1926. Serial No. 123,596.

This invention has reference to an alloy steel and has for its principal object to provide an improved alloy steel which shall be highly resistant to corrosion so as to be substantially rust-proof and which shall be tough, hard, malleable, readily workable and consequently suited for all general purposes such as for cutlery, dies, castings, valves, etc.

The property of chromium, when included in a steel alloy, of resisting staining and corrosion is well-known, and various alloys including chromium for this purpose have been proposed. Such alloys have been, generally speaking, capable of some particular use only (such for example as cutlery) and have even when employed for such purpose possessed some inherent disadvantage.

I have discovered that an alloy comprising iron, chromium, nickel, silicon, copper, zirconium, titanium and carbon is capable of use for all general purposes, is practically rust-proof under all ordinary conditions and can be hardened, forged, tempered and in short subjected to whatever treatment or operation is required for obtaining the article or apparatus in view. Thus when cutlery is to be made from this alloy it can be hardened, tempered and polished as desired and will take a sharp cutting edge.

My improved alloy being capable of such varied uses can have the proportions of its constituents varied within considerable limits and I have found it possible to work within the following ranges, viz:—

|                         | Per cent.    |
|-------------------------|--------------|
| Chromium                | 3 to 9       |
| Nickel                  | 1 to 12      |
| Silicon                 | 1 to 6       |
| Copper                  | 1 to 16      |
| Zirconium               | 0.5 to 6     |
| Titanium                | 0.5 to 4     |
| Carbon                  | 0.10 to 0.40 |
| and the remainder iron. |              |

For the majority of uses, however, I find that a narrower range of proportions can be stated, such for instance as

|                             | Per cent.  |
|-----------------------------|------------|
| Chromium                    | 5 to 9     |
| Nickel                      | 1 to 4     |
| Silicon                     | 1 to 4     |
| Copper                      | 1 to 3     |
| Zirconium                   | 0.5 to 2   |
| Titanium                    | 0.5 to 2   |
| Carbon                      | 0.1 to 0.4 |
| 55 with the remainder iron. |            |

The proportions will, of course, vary according to the article to be made or the use to which the alloy is to be put, but for guidance I will give hereinafter some typical examples which I have found from experience to be eminently satisfactory. Thus I have used for castings—

|                         | Per cent. |
|-------------------------|-----------|
| Chromium                | 8.75      |
| Nickel                  | 3.        |
| Copper                  | 1.        |
| Silicon                 | 1.5       |
| Carbon                  | 0.2       |
| Zirconium               | 0.75      |
| Titanium                | 0.5       |
| and the remainder iron. |           |

For blanking dies a higher percentage of copper and silicon is desirable and for this purpose the following are my preferred proportions—

|                         | Per cent. |
|-------------------------|-----------|
| Chromium                | 8.5       |
| Nickel                  | 2.        |
| Copper                  | 3.1       |
| Silicon                 | 2.1       |
| Carbon                  | 0.3       |
| Zirconium               | 1.        |
| Titanium                | 0.5       |
| and the remainder iron. |           |

For valves I prefer to use the following:—

|                         | Per cent. |
|-------------------------|-----------|
| Chromium                | 8.5       |
| Nickel                  | 2.5       |
| Copper                  | 2.1       |
| Silicon                 | 2.1       |
| Carbon                  | 0.3       |
| Zirconium               | 1.        |
| Titanium                | 0.5       |
| and the remainder iron. |           |

For cutlery I find the following proportions are most suitable:—

|                         | Per cent. |
|-------------------------|-----------|
| Chromium                | 8.75      |
| Nickel                  | 3.        |
| Copper                  | 1.        |
| Silicon                 | 2.        |
| Carbon                  | 0.4       |
| Zirconium               | 1.        |
| Titanium                | 1.        |
| and the remainder iron. |           |

My improved alloy steel is also useful for the manufacture of linings for ice-boxes, meat-hooks, choppers, golf stick heads, etc.

and for such purposes the following is the formula I prefer:—

|             | Per cent. |
|-------------|-----------|
| Chromium    | 8.5       |
| 5 Nickel    | 3.1       |
| Copper      | 2.5       |
| Silicon     | 2.5       |
| Carbon      | 0.15      |
| Zirconium   | 1.75      |
| 10 Titanium | 1.        |

and the remainder iron.

It is to be understood that all the above are given by way of example only and are 15 not to be considered restrictive. Broadly speaking, the inclusion of the copper, nickel, chromium and carbon mainly affects the physical properties of the resultant alloy

while the zirconium, silicon and titanium appear to act as deoxidizing agents. It will be 20 noticed particularly that copper is included in all the examples and I regard this as an essential and important ingredient.

When given a perfect melt a steel is produced of high resistance to all corrosion producing agents at the same time possessing hardness, toughness and high tensile strength.

The parts mentioned herein are by weight. What I claim and desire to secure by Letters Patent is:—

An alloy steel comprising chromium 8.75 per cent, nickel 3 per cent, copper 1 per cent, silicon 1.5 per cent, carbon 0.2 per cent, zirconium 0.75 per cent, titanium 0.5 per cent, with the remainder iron.

JOHN THOMAS WHITELEY.